

No. 897,842.

PATENTED SEPT. 1, 1908.

J. F. MONNOT.

PROCESS OF MAKING BIMETALLIC INGOTS, PLATES, SHEETS, TUBES, WIRES,  
AND LIKE PRODUCTS.

APPLICATION FILED MAY 23, 1905.



Attest:

John F. Monnot  
John F. Monnot

Inventor:

JOHN FERREOL MONNOT

by Dickson, Brown, Raegener & Bruner

Atty.

# UNITED STATES PATENT OFFICE.

JOHN FERREOL MONNOT, OF NEW YORK, N. Y., ASSIGNOR TO DUPLEX METALS COMPANY, OF NEW YORK, N. Y., A CORPORATION OF NEW YORK.

## PROCESS OF MAKING BIMETALLIC INGOTS, PLATES, SHEETS, TUBES, WIRES, AND LIKE PRODUCTS.

No. 897,842.

Specification of Letters Patent.

Patented Sept. 1, 1908.

Application filed May 23, 1905. Serial No. 261,740.

To all whom it may concern:

Be it known that I, JOHN FERREOL MONNOT, a citizen of the United States, and resident of the borough of Manhattan, city, county, and State of New York, have invented certain new and useful Improvements in Processes of Making Bimetallic Ingots, Plates, Sheets, Tubes, Wires, and Like Products, of which the following is a specification accompanied by drawings.

This invention relates to improvements in processes in making bi-metallic ingots, plates, sheets, tubes, wires, and like products, and its objects are to improve upon such processes and prevent waste, with a reduction of cost in the preparation and handling of the material to be operated upon.

According to this invention the products consist of bi-metals such as steel and copper, steel and brass, steel and silver and other combinations of ferrous metals with non-ferrous metals which are ductile, high-melting and of a generally copper-like character. The stated non-ferrous metals have high melting points and may therefore be worked with steel at steel-working temperatures, brass and silver being like copper in this respect as well as in others. Ingots of any required dimensions may be produced in accordance with this process and the proportions of the elements entering into the composition of the ingots may be exactly determined and maintained throughout the finishing processes. Once an ingot, for instance, is produced, the metals comprising it are so welded together that it is impossible to separate them either mechanically or by means of heat. They form a homogeneous mass that may be rolled into sheets or drawn into wires like a single metal.

Further objects of the invention will hereinafter appear, and to these ends the invention consists of a process for manufacturing bi-metallic ingots, plates, sheets, tubes, wires, and the like, substantially as herein-after fully described and claimed in this specification.

Suitable apparatus for carrying out the process is shown in the accompanying drawings, in which,—

Figure 1 is a horizontal sectional view of a suitable mold for carrying out the process; Fig. 2 is a longitudinal sectional elevation of the same; Fig. 3 is a transverse sectional elevation of the same; Fig. 4 is an enlarged detail transverse sectional view, partly broken away; Fig. 5 is an enlarged detail plan view of one of the ends for the mold; and Fig. 6 is a transverse sectional view of Fig. 5.

I have found that excellent qualities of bimetals may be made by first electro-depositing the coating metal on a suitable core of a different kind of metal from the coating and then welding the two metals together by means of heat and high compression.

The core metal, preferably steel or iron, in the form desired, as an ingot, bloom, billet or slab is first perfectly cleaned and the coating metal is deposited electrically on it in a layer of sufficient thickness to obtain the proportion desired between the core and coating metals. If, for instance, a steel slab about three inches thick is used for the core, an electro-deposit of copper of about one-half inch in thickness on each side of the core should be made in order to produce a 25 percent. finished bi-metal.

An electrodeposited coating of copper on steel though in itself crystalline, porous and of little mechanical strength with no more than an adherence to the base metal, nevertheless is in absolute molecular and metallic contact with such base on all abutting surfaces of copper and steel, the copper crystals being deposited on the steel surface in absolute contact therewith. The particles or crystals of the copper in the coating are also in similar absolute contact with each other. An absolute contact of copper and steel is difficult to secure by ordinary methods since copper at common casting temperatures does not "wet" steel nor do the solid or plastic metals readily contact at ordinary metal working temperatures with an absolute metallic contact. It is also difficult to secure such a contact between solid or plastic copper and a similar body of copper, copper being a non-welding metal. Absolute metallic contact of the two metals is very desirable to attain in forming steel-copper bimetals since thereby the coating may be given a degree of coherence to the base, as distinguished from a mere adherence. After the electro-deposit of the coating metal has been produced, the coated billet is then heated to the required temperature in a suitable furnace under conditions precluding oxidation. The heated billet at the required temperature is

55

60

65

70

75

80

85

90

95

100

105

then submitted to a high pressure by suitable means in order to compress the two metals on all their surface of contact and thus obtain a perfect weld. The bi-metallic billet 5 thus obtained can afterwards be reheated and rolled into any desired finished product, such as plates, sheets, tubes, wire, and the like. For producing bi-metallic plates and sheets, I prefer to use a rectangular billet or 10 slab of the desired metal for the core, which I preferably coat on the two flat sides. It is then heated as described and pressed between two well planed steel plates or heated in a suitable die. In the initial electrocoating 15 there is secured a coating of the full thickness desired and in metallic contact with the base, but this coating is weak, porous and crystalline, with no great adherence to the base. In the subsequent heating and press- 20 ing, in the described manner, this coating is rendered dense, impervious and strong while the adherence to the base is converted into a coherence sufficient to permit the joined metals to be coextended and otherwise worked 25 like one metal.

For producing wire a round billet is preferably used for the core. After the coating metal has been deposited on the core by any well known process the billet is heated and 30 preferably pressed in a suitable die. One form of die which is made especially for carrying out this process is illustrated in the drawings, although any suitable form of apparatus may be used. This die is made in 35 two parts *a* and *b* in which are cut ogival or Gothic grooves. The bottom part *a* is preferably fixed but the top *b* may move between the two side plates *c*. The dies *a* *b* and side plates *c* forming the mold, together with the 40 ends *s* are placed in a suitable hydraulic press which will hold the bottom *a* and side plates *c* firmly, leaving the top die *b* free to move.

The prepared and heated cylindrical billet is laid in the groove of the bottom piece *a*, 45 then the top piece *b* is placed in position and the arm of the press is brought to bear upon the block *D*, thereby forcing downwards the die *b* and compressing the billet from a round to an ogival form.

50 This form of die has the advantage of transmitting equal pressures on all the surfaces of the billet and thereby producing a perfect weld of the core with the coating metal. The

Gothic form is also advantageous for the subsequent rolling of the billet into bars, rods, 55 etc.

The end pieces *s* fit into the dies *a* and *b*, and therefore by preference have the configuration of the internal contour of such dies. Said pieces *s* are provided with axial longitudinal openings for the porter bar of the 60 ingot.

Obviously this process may be carried out in any suitable apparatus, and equivalent steps may be substituted for some of those 65 described, therefore, without enumerating equivalents,

I claim and desire to obtain by Letters Patent the following:

1. The process of producing bodies of unlike metals welded together which consists in electrically depositing on a core of ferrous metal a coating of a softer, ductile high-melting copper-like metal workable at steel working temperatures, heating core and coating 75 together, and while at a suitable temperature compressing them together by a transverse pressure upon all abutting surfaces. 70

2. The process of producing bodies of unlike metals welded together which consists in 80 depositing electrically a coating of a softer, non-ferrous, high melting, copper-like metal upon a core of a ferrous metal, heating the coated core to a suitable temperature and while at such temperature pressing the coated 85 core between dies adapted to produce pressure upon all abutting surfaces of the joined metals.

3. The process of producing bodies of copper welded to steel which consists in electrically depositing a coating of copper upon steel, said coating corresponding to the thickness desired in the finished article, heating the coated core to a suitable temperature and while at such temperature pressing the coated 95 core between dies adapted to produce pressure upon all abutting surfaces of the joined metals. 90

In testimony whereof I have signed this specification in the presence of two subscr- 100 ing witnesses:

JOHN FERREOL MONNOT.

Witnesses:

OLIN A. FOSTER,  
A. L. O'BRIEN.